

J. L. Gilliland,

33 sheets, sheet 1.

Glass Mold

No. 9,184.

Patented Aug. 10, 1852.



J. L. Gilliland,

3 Sheets, Sheet 2.

Glass Mold.

No. 9,184.

Patented Aug. 10, 1852.



J. L. Gilliland,

38heet, Sheet 3.

Glass Mold.

No 9,184.

Patented Aug. 10, 1852.



# UNITED STATES PATENT OFFICE.

JOHN L. GILLILAND, OF NEW YORK, N. Y.

## MANUFACTURE OF GLASS LENSES.

Specification of Letters Patent No. 9,184, dated August 10, 1852.

*To all whom it may concern:*

Be it known that I, JOHN L. GILLILAND, of New York, N. Y., have invented a new and useful Manufacture of Molded and Pressed Dioptric Lenses, and that the following is a full, clear, and exact description thereof, reference being had to the accompanying drawings, making part of this specification.

10 The dioptric lens heretofore and at the present time in use for sea lights and for other lights requiring great intensity being constructed of single zones or rings made up of segments according to the diameter 15 of the required lens has induced a belief that glass could not be prepared without incurring the expense of grinding and polishing the curved surface and that economy dictated a method of manufacturing, embracing a center and zones or segments.

An examination into the necessity daily shown for the more general use of a dioptric lens to the purpose of a sea light including under that name either revolving or stationary coast light, bay light, bar light, ship signal light, deck and between deck light, port light and all other light for ships, tide light, floating light and coast, harbor and river light, generally, and also a land light, 25 including under that name railway locomotive light, carriage light, ferry light, and as applied to architectural purposes, and in fact to any purpose where an intensity of light is required, induced me to examine the 30 method of construction of the "built-up lens" and essay at least to reduce the expense without reducing the strength of the light.

Commencing with the suggestions of Buffon that a spherical body from its thickness absorbs light in proportion to its density and that a sectional figure of any required shape and thickness could be cast of vitrified material or glass and ground in 40 steps or concentric zones to produce a lens as executed with partial success by the Abbé Rochon, from the expense incident to the accuracy required in grinding and polishing the steps or zones; although I could fully 45 appreciate the lens of Buffon it was beyond the reach of the million by reason of the cost. The experiments of the Abbé Rochon were, however, useful in preparing the way for the manufacture of the dioptric lens in 50 separate pieces which was subsequently accomplished by the ingenious Fresnel, after

the suggestions of Condorect, known as the "annular band lens" at the present time in use in several light houses, in which the spherical aberrations are nearly corrected by 60 making the foci of each zone to coincide.

Although of great utility, the enormous expense of making the annular band lens of Fresnel, in which, not only must each separate piece have its surfaces formed with 65 great accuracy but all the several pieces must be fitted to each other so that when put together they shall constitute a perfect whole, has limited the use of this otherwise valuable and desirable invention to a very 70 few localities.

The object of my invention is to produce a dioptric lens which shall present all the practical advantages of the annular band lens of Fresnel and at the same time so 75 cheap as to admit of being applied to all purposes requiring intensity of light, and to the end my invention consists in a new manufacture of dioptric lenses made in one or several pieces molded and pressed, the form required for the surfaces, and (when made of several pieces) the required fit of the several parts being produced by giving the reversed required form to the metal molds in which the molten glass is to be put and 80 into and by which it is to be pressed the pressure to be applied being sufficient to produce the required surfaces and angles.

The mode of procedure which I have adopted with success is as follows, reference 90 being had to the accompanying drawings and marked Nos. 1, 2 and 3.

In the accompanying drawings No. 1, *a*, represents a circular mold to receive the melted glass; *b*, is a follower which rests on 95 the mold as shown at *b'*, *b''*. *c'*, is a plunger which fits into the follower *b*, and which is intended to spread the melted glass uniformly into the mold *a*, by pressure; the mold, plunger and follower as described being well known to glass workers. The mold may be made of any figure required and the follower and plunger will be made to correspond with the mold. The mold *a*, instead of having the concentric central lens and 100 rings as shown, may present a plane surface and the melted glass laid thereon and the follower *b*, placed as hereinbefore described, the plunger *c'* having on it the rings and figures as shown in the mold *a*, by pressure 105 upon the melted glass as already described upon the melted glass as already described 110 will produce the required figure. The shape

of the mold may be changed to any figure whether convex or concave with the central zones or rings. *d*, is a section of *a*, taken at the dotted lines *e*, *f*, and shows in section 5 the figure of a lens.

The mold instead of being made of one piece as at *c*, *a*, may be made sectionally of as many separate rings or zones as there are designed to be rings or zones in the lens or 10 otherwise sectionally divided according to convenience, a suitable allowance in the diameter of each being made for the increased aggregate diameter by reason of the parts being distinct, and in such cases the molds 15 for the separate rings and zones being laid together and secured in their proper order, will form the entire mold while the interstices left between the separate pieces will answer the same purpose as the holes in the 20 angles of the zones, subsequently described, viz.: to suffer the air to escape when the pressure is applied.

If it should be desired (as it may be in the case of very large lights) to cast the lens 25 itself in sections the several sections may be molded and pressed as described above, and then the whole cemented together in the usual way.

*g*, shows a concentric dioptric lens corresponding with the molds *a*, and is set in a 30 frame ready for use. The frame may be made of any suitable metal.

No. 2. *h*, shows three sides of a figure, of which *i* is a sectional view taken at *i'*, *i''*, 35 containing six sides, each lens having a convex center and several sections of zones or rings. *K* shows a figure made in three pieces *k'*, *k''*, *k'''*, which will require three separate molds or it may be made in 40 one mold. The six sided figure *h*, is illustrated to show that it may be added to or diminished in the number of lens to be used. The several lenses to make up the required figure may be set in a metal frame; 45 the cap *l*, may be varied in shape and may be made of any suitable metal.

No. 3, shows a dioptric cylinder *m*, applicable to the purposes of a lantern containing several zones or rings with annular bands of regular and irregular widths 50 which can be varied at pleasure and may be manufactured of any length or circumference. *n*, shows a transverse vertical section of *m*, as applied to the purposes of a hanging or hand lantern with a stand lamp, top 55 and ring attached.

If required, each lens may be made of one or many zones or concentric rings with the central lens according to the diameter 60 the lens or segment of a lens being produced as shown and described, by pressure, in a mold with or without fire polishing a process well known among glass workers.

To promote focal intensity and to prevent 65 the absorption of light it will be obvious

that each lens should be manufactured as thin as the size and number of concavities and convexities will permit. It is not essential to lay down any rule for thickness or for the size as the intensity will be decreased by density, and that, therefore, the thickness will be governed by the extent of surface required. 70

In the making of dioptric lenses, sharpness at the angles of the zones is of the 75 utmost importance, and to effect this important object it may be found necessary to make the parts of the mold which are to form the angles of the zones with apertures (so small as to be nearly invisible to the 80 naked eye) for the escape of air from the cavity of the mold, otherwise atmospheric air may be confined in such cavities, and when pressure is applied, the air thus confined will prevent the glass from entering 85 and assuming the required form of the sharp angles of the mold.

The holes should be very small and at such distances apart as to insure the escape 90 of the air.

When that part of the mold which forms the curved surfaces of the zones is made in sections sufficient space can be left between the different zones for the escape of the air. 95

In the manufacture of the dioptric lens invented by me I use a metal mold or molds as I have already described, the reverse of the figure to be produced and which will require accuracy in construction and finish. 100

The melted glass being prepared in the usual way well known to glass workers, is to be put into the mold and the same process or labor is required in producing a lens, as is observed in molding by pressure any other article from melted glass. The quality 105 of the glass is not essential, but as light is always lost even in passing through the most transparent body, it will be more economical as well as more useful to employ a good quality of glass and as white as possible, as white glass will permit the more free passage of light, and with more brilliancy than an inferior quality and of less whiteness. 110

In describing my invention as a manufacture and its adaptation to the various uses hereinbefore mentioned it is not essential to detail the peculiar way in which sea lights are used nor the adaptation of the dioptric lens to the several purposes spoken of other than sea lights nor the many sided lanterns, whether stationary or revolving, in use, nor the peculiar shape of the case or shell, nor the lamp, nor the many ways in which light may be refracted as any person essaying to use or manufacture my dioptric lens will be prepared with the necessary means, and I therefore consider it unnecessary to detail in words or to show in the drawings the manner of constructing the 115 120 125 130

different kinds of apparatus in use for that purpose, I therefore disclaim the invention of any apparatus connected with the use of the dioptric lens.

5 What I claim as my invention and desire to secure by Letters Patent is—  
The manufacture of dioptric lenses of

glass in steps or rings by pressure in metallic molds, substantially as specified.

JOHN L. GILLILAND.

Witnesses:

CANSTEN BROWN,  
Wm. H. BISHOP.